

H. W. BUTTERWORTH.  
APPARATUS FOR COATING METAL PLATES WITH TIN AND OTHER METALS.  
No. 68,351. Patented Sept. 3, 1867.



Witnesses;

Wm. Abbot Slade  
S. H. Gorham Godwin

Inventor;

H. W. Butterworth  
By his Atty  
J. H. Hawley

# United States Patent Office.

H. W. BUTTERWORTH, OF PHILADELPHIA, PENNSYLVANIA,

*Letters Patent No. 68,351; dated September 3, 1867.*

## IMPROVED APPARATUS FOR COATING METAL PLATES WITH TIN AND OTHER METALS.

The Schedule referred to in these Letters Patent and making part of the same.

TO ALL WHOM IT MAY CONCERN:

Be it known that I, H. W. BUTTERWORTH, of Philadelphia, Pennsylvania, have invented certain Apparatus for Coating Metal Plates with Metal; and I do hereby declare the following to be a full, clear, and exact description of the same.

My invention consists of certain apparatus, fully described hereafter, by which a smooth coating of metal of uniform thickness may be quickly imparted to metal plates.

In order to enable others skilled in the art to make and use my invention, I will now proceed to describe its construction and operation, reference being had to the accompanying drawing, which forms a part of this specification, and in which—

Figure 1 is a vertical section of my apparatus for coating metal plates with metal, and

Figure 2 a plan view.

A is a furnace, containing a suitable fire-place, and supporting the pan B, which, in the present instance, consists of a dish made in the arc of a circle and resting on the walls of the furnace, within which the greater portion of the pan is contained, as seen in fig. 1. On the bottom of the pan is a projection or apron,  $b^2$ , the upper surface of which is curved, and at one end of this apron are two rollers,  $a$  and  $a'$ , and at the opposite end two similar rollers,  $b$  and  $b'$ , the journals of these rollers turning in the opposite ends of the pan, and the rollers being geared together. A pinion on the roller  $a$  gears into a pinion,  $d$ , on a spindle,  $e$ , which passes through and turns in one end of the pan; a pinion on the roller  $b$  gearing into a pinion,  $d'$ , on a similar spindle,  $e'$ , and the two pinions being so geared together, by belts or otherwise, that the several rollers may revolve in the directions indicated by their respective arrows.

In coating metal plates with metals, such as sheet-iron plates with tin, it has been the practice to dip the former, properly prepared, into a molten mass of the latter, an operation which frequently results in an unequal distribution of the tin, parts of the plate having consequently a waved appearance.

In using my invention a body of tin is maintained in a molten state in the pan, by the fire in the furnace A, and the properly prepared sheet iron  $x$  is passed over and in contact with one edge of the pan, and down the guide-plate  $y$  towards the rollers  $b$  and  $b'$ , by which the plate is drawn forward, pushed over the curved surface of the apron  $b^2$  to the rollers  $a$  and  $a'$ , by which the plate is withdrawn from the molten tin preparatory to its removal, these latter rollers imparting an even coat of uniform thickness to the plate. Between the opposite ends of the pan B, I place a detachable vessel or other object,  $h$ , which should be of such form and dimensions as to cover as much as possible of the molten tin without interfering with the rollers, thereby preventing undue oxidation of the molten metal. Although I prefer the use of two pairs of rollers, one for drawing the plate  $x$  into the molten metal, and the other pair for withdrawing it from the same, the latter pair only may be used, the plate in which case is pushed through the molten metal to the rollers  $a$  and  $a'$ , which complete the operation.

I claim as my invention, and desire to secure by Letters Patent—

1. Rollers  $a$  and  $a'$  combined with a pan containing molten metal, substantially as and for the purpose herein set forth.
2. The pan B in combination with the rollers  $a$  and  $a'$  and  $b$  and  $b'$ , geared together so as to operate simultaneously, as described, for the purpose specified.
3. The arrangement of the curved apron  $b^2$ , in the bottom of the pan B, in respect to the rollers  $a$  and  $a'$  and  $b$  and  $b'$ .

In testimony whereof I have signed my name to this specification in the presence of two subscribing witnesses.

H. W. BUTTERWORTH.

Witnesses:

JOHN WHITE,  
W. J. R. DELANY.